

Patented Nov. 1, 1932

1,885,524

# UNITED STATES PATENT OFFICE

ARTHUR LAZAR, OF ASSOCIATED, CALIFORNIA, ASSIGNOR TO ASSOCIATED OIL COMPANY, OF SAN FRANCISCO, CALIFORNIA, A CORPORATION OF CALIFORNIA

## PROCESS FOR TREATING HYDROCARBON OILS

No Drawing.

Application filed December 17, 1927. Serial No. 240,931.

This invention relates to an improved process for treating hydrocarbon oils to produce an oil with new and valuable characteristics.

5 Stability towards oxidation and thermal decomposition are characteristics very desirable in oils such as those used in transformers, turbines and in internal combustion engines.

10 It is therefore the object of this invention to treat certain distillate fractions in such a manner that the product resulting therefrom exhibits a vast improvement in the desired characteristics. This process consists essentially in the treatment of lubricating distillates and the like with a selective solvent, redistilling or reducing the oil, with or without previous neutralization, to attain the desired physical characteristics, and the particular manner in which the adsorbent material is utilized for decolorizing and removing other impurities.

15 Heretofore, in the production of such oils it has been the general practice among refiners to select distillate fractions of the approximate physical characteristics desired, reducing the distillate until the oil has the proper viscosity or flash; then subjecting the distillate to the usual acid treatment, and 20 after neutralizing with a caustic solution, treating with some adsorbent material such as clay to remove decolorizing matter and other impurities. It has been found that oils of certain origin produced in this manner, especially the lubricating oils, do not show 25 sufficient stability toward oxidation and thermal decomposition.

25 In the treatment which is the subject of this invention, certain hydrocarbon fractions are selected whose physical characteristics most nearly approach those desired in the finished oil.

30 These fractions are then treated with a selective solvent, in which the unsaturated and aromatic compounds are dissolved and then are removed by gravity separation. The undissolved portion, the so-called raffinate is then reduced to the desired viscosity and flash and the reduced oil treated with an adsorbent decolorizing material. It is essential

35 to maintain the sequence of operations as described in order to obtain finished products of high qualities. It has been found that when reduction of the oil is carried out prior to the treatment with the selective solvent, 40 certain hydrocarbons break down under heat into forms in which they are objectionable in the lubricant but not soluble in the selective solvent later. On the other hand, if the un- 45 reduced hydrocarbon oil is first treated with a selective solvent, the components which are liable to break down and form the objectionable and insoluble hydrocarbons mentioned before, are removed and only those of 50 a more stable nature remain during the reduction which follows. It is of importance 55 to note that the same lubricating stocks treated by the same operations but in a different sequence as described by carrying out the reduction before the treatment with the 60 selective solvent will show much inferior 65 qualities in use. Furthermore, it can be 70 proved that mere laboratory testing is not sufficient for characterizing the real value of 75 oils which have to perform under severe conditions, as, for example, in an internal combustion engine. The two products processed 80 by the same operations but in a different sequence of the individual steps usually will 85 show very similar physical properties. Upon 90 more thorough tests of performance under the most severe conditions in a stationary internal combustion engine and in road tests, the oil processed in the proper sequence of 95 operations as described above will perform much better than the one which had been reduced previous to the treatment with the 100 selective solvent. The latter one, submitted to a test run in the motor shows high consumption, high carbon deposition and gummy or resinous deposits on the moving parts of the engine, whereas the product obtained by the proper method treating with the selective solvent, reducing after the treatment and decolorizing the reduced oil will be found to be an excellent lubricant.

105 Of all the substances which show selective dissolving properties of hydrocarbon oils, liquid sulphur dioxide is known to be the most suitable and effective. As far as the 110

treatment with this solvent is concerned, the treated oil naturally is bound to show a slight acidity due to traces of the solvent retained in the so-called raffinate. In the majority of cases this slight acid reaction might deteriorate the color of the bottoms during the following reduction and also endanger the reducing equipment by corrosion. For this reason, a neutralization previous to the reduction is advisable. It might be mentioned that this neutralization has no effect at all on the internal qualities of the finished product but is only recommended for getting a good final color. As neutralizing agents, all kinds of chemicals either in gaseous, liquid or solid form, can be used, the kind of chemical and manner of application depending chiefly on the equipment available. It is also possible to carry out the reduction in the presence of the neutralizing agent. As suitable neutralizing agents may be mentioned ammonia in gaseous form or solution, the oxides and hydroxides of the alkaline earth metals, aluminum oxide and hydroxide and other adsorbent materials like clay. Those latter ones not only act as neutralizing agents but also have a high adsorptive power for colored materials, thus combining a considerable decolorizing effect with the neutralizing action. It is evident that the use of such kinds of adsorptive materials for neutralization, previous to the reduction, will make it possible to cut down the amount of adsorbent clay to be applied to the reduced oil in the last step of the process as heretofore described.

Having now more particularly described this invention, the application of this process should only be restricted and defined by the hereinafter appended claims.

40 What I claim is:

1. The process of treating hydrocarbon oils which comprises treating the lubricating fractions with liquid sulphur dioxide, separating the undissolved portion from the dissolved portion, and reducing by distillation the undissolved portion in the presence of an adsorbent decolorizing material.

2. The process of treating hydrocarbon oils which comprises treating the lubricating fractions with liquid sulphur dioxide, separating the undissolved portion from the dissolved portion, reducing by distillation the undissolved portion in the presence of an adsorbent decolorizing material, and removing the adsorbent material.

3. The process of treating hydrocarbon oils which comprises treating lubricating fractions with liquid sulphur dioxide, separating the undissolved portion from the dissolved portion, and reducing by distillation the undissolved portion in the presence of a neutralizing and decolorizing adsorbent material.

4. The process of treating hydrocarbon oils which comprises treating lubricating

fractions with liquid sulphur dioxide, separating the undissolved portion from the dissolved portion, reducing by distillation the undissolved portion in the presence of a neutralizing and decolorizing adsorbent material, and treating the reduced portion with further adsorbent decolorizing material.

5. The process of treating hydrocarbon oils which comprises treating lubricating fractions with liquid sulphur dioxide, separating the undissolved portion from the dissolved portion, reducing by distillation the undissolved portion in the presence of a neutralizing and decolorizing adsorbent material, and treating the reduced portion with further adsorbent decolorizing material of the same character.

ARTHUR LAZAR.

85

90

95

100

105

110

115

120

125

130